

July 6, 1971

K. H. J. BUSCHOW ET AL

3,591,428

BASIC SUBSTANCE FOR THE MANUFACTURE OF A PERMANENT MAGNET

Filed Nov. 26, 1968



## 1

3,591,428

### BASIC SUBSTANCE FOR THE MANUFACTURE OF A PERMANENT MAGNET

Kurt Heinz Jurgen Buschow, Pieter Aart Naastepad, Wilhelmus Antonius Johannes Josephus Velge, and Johannes Hendrikus Nicolaas van Vucht, Emmasingel, Eindhoven, Netherlands, assignors to U.S. Philips Corporation, New York, N.Y.

Filed Nov. 26, 1968, Ser. No. 778,981

Claims priority, application Netherlands, Dec. 21, 1967, 10  
6717442

Int. Cl. H01f 1/08

U.S. Cl. 148—31.57

12 Claims

#### ABSTRACT OF THE DISCLOSURE

A permanent magnet material is disclosed having a large intrinsic coercive force ( $I_H_c$ ) and thus strongly resistant to demagnetization and a large energy product  $-(BH)_{max}$ . This material consists of fine particles having permanent magnet properties and consisting essentially of a compound  $M_5R$  having a hexagonal crystal structure. M in this compound is cobalt or a combination of cobalt with one or more of the elements Fe, Ni, and Cu while R is a rare earth metal (which term includes Y) and/or Th. These particles are surrounded with a metallic layer.

The invention relates to a basic substance for the manufacture of a permanent magnet consisting of fine particles in themselves having permanent magnetic properties, the essential constituent being a compound of hexagonal structure the existence region of which is integral with the existence region of the compound  $M_5R$  in the system MR, wherein M designates Co or a combination of Co with one or more of the elements Fe, Ni and Cu and R designates one or more of the rare earth metals and/or Th. The rare earth metals are considered in this respect to include also the element Y.

Such basic materials are known from Dutch patent application No. 6608335 which has been opened for public inspection. They exhibit a high magnetic anisotropy in conjunction in most cases with a high magnetization.

Since a basic substance for the manufacture of permanent magnets consisting of fine particles of this basic substance must satisfy the requirement that the intrinsic coercive force  $I_H_c$  and the magnetization  $\sigma$  should be sufficiently high, the aforesaid  $M_5R$  compounds can be successfully employed to this end.

Such a known basic substance may be formed by fine particles of the compound  $SmCo_5$ . Depending upon the degree of deformation and size these particles may have an  $I_H_c$  of 10,000 oersted (oe.) and a  $\sigma_{24K}$  oe. of 90 ergs/g. oe. and an  $I_H_c$  of 10,000 oe.

A basic substance according to the invention is characterized in that the particles are surrounded by a metallic layer.

The term "metallic" is defined herein as "consisting of a metal, an alloy of metals or an alloy of one or more metals with one or more metalloids."

Such basic substances according to the invention, due to their being plated, exhibit an increase in the  $I_H_c$ .

The following values measured on  $SmCo_5$  are illustrative of this improvement in  $I_H_c$  of a basic substance according to the invention. The measurements are based on a non-

## 2

plated  $SmCo_5$  powder having an  $I_H_c$  of 6500 oe. After plating the following results were obtained:

|                                                  | $I_H_c$ oe. |
|--------------------------------------------------|-------------|
| 5 $SmCo_5$ plated with Ni-P                      | 17,000      |
| Sm <sub>5</sub> Co <sub>5</sub> plated with Ni-B | 11,000      |
| Sm <sub>5</sub> Co <sub>5</sub> plated with Co-P | 7,700       |
| Sm <sub>5</sub> Co <sub>5</sub> plated with Co-P | 7,700       |
| Sm <sub>5</sub> Co <sub>5</sub> plated with Sn   | 15,300      |
| Sm <sub>5</sub> Co <sub>5</sub> plated with Cu   | 9,300       |

The invention will be described with reference to the drawing in which the sole figure shows graphs relating the magnetic properties to the thickness of the metal layer.

It should be noted that the magnetization of the plated particles depends upon the thickness of the surrounding layer. As is indicated in the graph I of the  $\sigma_{25K}$  oe., as compared with that of non-plated basic material, first increases with an increasing thickness of the layer—which involves a longer plating time  $t$ —and then decreases. Graph II indicates the relationship between the  $I_H_c$  and the plating time  $t$ .

The invention furthermore relates to a method of manufacturing a basic substance of the kind set forth in as much as the layers consist of one or more metals of the EMF series nobler than Zn, alloyed or not alloyed with metalloids.

In this method the cast made by melting the constituents and by subsequent cooling is refined. The refinement is continued until the particles have the desired magnetic properties, for example, the desirable  $I_H_c$  and orientability.

The method according to the invention is characterized in that the particles are first etched, then washed, if necessary, and finally introduced into a bath containing a solution of salts appropriate for depositing chemically, or electro-chemically, the desired layer on the surface of the particles.

The following examples are illustrative.

#### EXAMPLE I

An Ni-P layer was applied to  $SmCo_5$  particles as follows:  $SmCo_5$  powder was etched by means of 1 N  $H_2SO_4$  in an ultrasonically vibrating vessel at a temperature between 20 and 50° C. for 60 seconds. At lower temperatures the period of etching must be longer. Then the acid was removed and the material was washed in cold water.

The powder was then introduced into a bath containing:

35 gms./liter of  $NiSO_4 \cdot 7H_2O$ ,  
30 gms./liter of amino-acetic acid,  
15 gms./liter of  $NaH_2PO_2 \cdot H_2O$ .

The pH value was 4.5 (to be adjusted with  $NH_4OH$ ) and the temperature was 50° C.

#### EXAMPLE II

The application of a Co-P layer to  $SmCo_5$  particles. First etching was carried out as described in Example I. The solution contained:

27.1 gms./liter of  $CoCl_2 \cdot 6H_2O$ ,  
45.3 gms./liter of  $NH_4Cl$ ,  
90 gms./liter of  $Na$ -citrate- $2H_2O$ ,  
9 gms./liter of  $NaH_2PO_2 \cdot H_2O$ .

By means of  $NH_4OH$  the pH value was brought to 8.5. At 75° C. the rate of growth of the layer thickness was 0.005  $\mu/min.$

### 3 EXAMPLE III

The application of an Ni-Co-P-layer. First etching was carried out as in Example I.

The composition of the solution was like that of Example I with the addition of 12 gms./liter of  $\text{CoSO}_4$ .

Plating was carried out at a pH value of about 7 and at a temperature of 60° C.

### EXAMPLE IV

The application of a Cu-layer. First etching was carried out as described in Example I.

The solution contained:

200 gms./liter of  $\text{CuSO}_4$ ,  
60 gms./liter of  $\text{H}_2\text{SO}_4$ .

Plating was carried out at a temperature of 20° C.

The invention furthermore relates to a permanent magnet made from the aforesaid basic substance. Such a magnet has a higher  $I_{\text{Hc}}$  than a magnet made from fine, non-plated particles of the same compound and will therefore exhibit an improved resistance to demagnetizing fields.

### EXAMPLE V

$\text{SmCo}_5$ -particles are surrounded by a metallic Cu-layer by means of "sputtering." For one hour, Cu was sputtered on to the  $\text{SmCo}_5$ , resulting in a Cu-layer having a thickness of  $0.24\mu$ .

The values of  $\sigma$  and  $I_{\text{Hc}}$  were raised from 91.5 to 93 erg/gr. oe. respectively from 6500 oe. to 9600 oe.

### EXAMPLE VI

$\text{SmCo}_5$ -particles were surrounded by an Ag-layer by means of a sputtering process of 1 hour, resulting in a layer of a thickness of  $0.36\mu$ .

The  $\sigma$ - and  $I_{\text{Hc}}$ -values were raised from 91.5 erg/gr. oe. to 94.5 erg/gr. oe. respectively from 6500 oe. to 10,100 oe.

A permanent magnet made from the basic substance according to the invention may also be anisotropic. Also this anisotropic magnet will exhibit a higher resistance to a demagnetizing field, while in addition the product  $(\text{BH})_{\text{max}}$  may be higher.

An example of an anisotropic permanent magnet according to the invention is a magnet consisting of  $\text{SmCo}_5$  particles plated with an Ni-P-layer. This magnet has a  $(\text{BH})_{\text{max}}$  of  $9 \times 10^6$  G oe. and  $I_{\text{Hc}}$  of 17,000 oe., whereas a magnet made from non-plated, but otherwise identical  $\text{SmCo}_5$  particles has a  $(\text{BH})_{\text{max}}$  of  $7 \times 10^6$  G oe. and an  $I_{\text{Hc}}$  of 6500 oe.

Particularly when an anisotropic permanent magnet is made from a basic substance according to the invention, the advantage of these substances is conspicuous. It is known that a basic substance for the manufacture of an anisotropic permanent magnet has to satisfy not only requirements with respect to a sufficiently high  $I_{\text{Hc}}$  and, which values are raised both by suitable plating, but also the requirement that in a magnetic field the particles should allow for satisfactory orientation. A measurement for the orientability of the particles is the ratio  $I_r/I_s$ , wherein  $I_r$  is the remanence and  $I_s$  is the saturation magnetization per unit of volume. It has been found that during the refining process for obtaining the fine particles after a given time the  $I_r/I_s$  drops. In order to attain optimum  $I_{\text{Hc}}$  values it is, however, necessary to continue the refining process for a given period of time. Unfortunately, the drop of the ratio  $I_r/I_s$  starts already before the optimum  $I_{\text{Hc}}$ .

Since, however, the basic substance plated in accordance with the invention has a considerably higher  $I_{\text{Hc}}$  than a comparable non-plated basic substance, a shorter period of the refining process may be chosen so that the  $I_r/I_s$  has

### 4

not yet, or has scarcely diminished. The resultant non-optimum  $I_{\text{Hc}}$  is then raised by the plating process to an extent such that the final  $I_{\text{Hc}}$  of the plated powder largely exceeds that of the non-plated particles. The advantage of the improved orientability of the particles becomes manifest in the higher  $(\text{BH})_{\text{max}}$  product of the magnet.

While the invention has been described with reference to particular examples and applications thereof, other embodiments will be apparent to those skilled in this art without departing from the spirit and scope of the invention which is defined in the appended claims.

What is claimed is:

1. A basic substance for the manufacture of a permanent magnet consisting of fine particles themselves having permanent magnetic properties, the essential constituent being a compound of hexagonal structure, the existence region of which is integral with the existence region of the compound  $M_5R$  of the system MR, wherein M is an element selected from the group consisting of Co, a combination of Co with at least one of the elements Fe, Ni and Cu, and wherein R is selected from the group consisting of at least one of the rare earth metals, Th, and the combination of Th with at least one of the rare earth metals, each said particles being coated with a layer of a metal which increases the coercive force of said particles.
2. A basic substance as claimed in claim 1 in which the M is Co, R is Sm and the metallic layer contains Ni.
3. A basic substance as claimed in claim 2 in which the nickel is alloyed with an element selected from the group consisting of P and B.
4. A basic substance as claimed in claim 2 in which the metallic layer consists of nickel.
5. A basic substance as claimed in claim 1 in which M is Co, R is Sm and the metallic layer contains Co.
6. A basic substance as claimed in claim 5 in which the cobalt is alloyed with an element selected from the group consisting of P and B.
7. A basic substance as claimed in claim 5 in which the metallic layer consists of Co.
8. A basic substance as claimed in claim 1 in which M is Co, R is Sm and the metallic layer contains Sn.
9. A basic substance as claimed in claim 8 in which the Sn is alloyed with an element selected from the group consisting of Zn and Cd.
10. A basic substance as claimed in claim 8 in which the metallic layer consists of Sn.
11. A basic substance as claimed in claim 1 in which M is Co, R is Sm and the metallic layer consists of Cu.
12. An anisotropically magnetized permanent magnet consisting of magnetically oriented particles consisting essentially of a basic substance as claimed in claim 1, said magnet having a higher  $(\text{BH})_{\text{max}}$  value than a like magnet consisting of particles of the same composition without a metallic layer thereover.

### References Cited

#### UNITED STATES PATENTS

- |           |        |                     |            |
|-----------|--------|---------------------|------------|
| 2,967,794 | 1/1961 | Coxe -----          | 148—31.57X |
| 3,424,578 | 1/1969 | Strnat et al. ----- | 75—213     |
| 3,463,678 | 8/1969 | Becker -----        | 148—105    |

#### FOREIGN PATENTS

- |         |         |                   |           |
|---------|---------|-------------------|-----------|
| 736,923 | 6/1966  | Canada -----      | 204—23    |
| 6608335 | 12/1967 | Netherlands ----- | 148—31.57 |

HYLAND BIZOT, Primary Examiner

G. K. WHITE, Assistant Examiner

U.S. CL. X.R.

148—103; 204—23